

April 13, 1965

HAJIME NAKAMURA

3,178,279

NITRIDE BEARING LOW-MANGANESE DUCTILE STEEL

Filed April 20, 1962

5 Sheets-Sheet 1

T1Q-1.

Q.T.: 930°C x 1 hr, Oil-Cooled; 650°C x 1.5 hrs, Air-Cooled

N: 930°C x 1 hr, Air-Cooled



INVENTOR  
HAJIME NAKAMURA

BY

*Molte & Molte*

ATTORNEY

April 13, 1965

HAJIME NAKAMURA

3,178,279

NITRIDE BEARING LOW-MANGANESE DUCTILE STEEL

Filed April 20, 1962

5 Sheets-Sheet 2

T1 Q-2.



INVENTOR  
HAJIME NAKAMURA  
BY  
*Nolte & Nolte*

ATTORNEY

April 13, 1965

HAJIME NAKAMURA

3,178,279

NITRIDE BEARING LOW-MANGANESE DUCTILE STEEL

Filed April 20, 1962

5 Sheets-Sheet 3

71-2-3.

N: 930°C x 1hr, Air-Cooled  
Q.T.: 930°C x 1hr, Oil-Cooled;  
650°C x 1.5 hrs, Air-Cooled



INVENTOR  
HAJIME NAKAMURA

BY

*Nolle & Nolle*

ATTORNEY

April 13, 1965

HAJIME NAKAMURA

3,178,279

NITRIDER BEARING LOW-MANGANESE DUCTILE STEEL

Filed April 20, 1962

5 Sheets-Sheet 4

7194.

A.B: 930°C x 1 hr, Air-Cooled

A'.B': 930°C x 1 hr, Oil-Cooled;  
650°C x 1.5 hrs, Air-Cooled



INVENTOR.

HAJIME NAKAMURA

BY

*Molte & Molte*

ATTORNEY

April 13, 1965

HAJIME NAKAMURA

3,178,279

NITRIDE BEARING LOW-MANGANESE DUCTILE STEEL

Filed April 20, 1962

5 Sheets-Sheet 5

T 19-5.



3% Nital Etch 100 X  
Ductile Steel LMn 1, 930°C x 1 hr., Oil-Cooled;  
650°C x 1.5 hrs., Air-Cooled  
ASTM Ferrite Grain Size Number, No. 12

T 19-6.



400 X

Same Specimen as above

INVENTOR:

BY Hajime Nakamura  
Holle & Holle  
Attorneys

# United States Patent Office

3,178,279  
Patented Apr. 13, 1965

1

3,178,279  
NITRIE BEARING LOW-MANGANESE  
DUCTILE STEEL

Hajime Nakamura, Tokyo-to, Japan assignor to Ishikawa-  
jima-Harima Jukogyo Kabushiki Kaisha, Tokyo-to,  
Japan, a company of Japan

Filed Apr. 20, 1962, Ser. No. 189,211

Claims priority, application Japan, May 16, 1961,  
36/17,371

6 Claims. (Cl. 75—124)

The low-Mn grade steels are gaining popularity in recent years for use as structural steel. In such application, however, the notch transition temperature must be low, and for that purpose, the ferrite grain size must be uniformly refined. For some time it has been assumed that aluminum oxide is effective for grain refinement and acquiring uniformity, but according to theories precipitated aluminum nitride is more effective in that respect; this theory is in agreement with the discoveries of the present inventor.

Thus it is the object of the present invention to provide low-Mn steels having refined and uniform granular structure, which are best suited for serving as structural steels at low temperatures. Although the low-Mn steel of the present invention exhibits markedly improved ductility due to the presence of appropriate amounts of aluminum nitride as a precipitate, it is in practice not feasible to provide the accurate amounts of aluminum and nitrogen needed for the formation of the desired amounts of aluminum nitride. In every case in practice, either nitrogen or aluminum will be in excess with respect to the other component. When nitrogen is in excess, it will exert a detrimental effect on the ductility of the steel leaving free nitrogen therein; excess of aluminum, on the other hand, dissolved as solid solution, counteracts the improvement in ductility, too, by coarsening the granular structure. Consequently, if low-Mn steel is to be produced, having a refined and uniform granular structure, the amount of free nitrogen must be limited as much as possible, leaving aluminum in excess over the amount required for the formation of aluminum nitride; however, the amount of metallic aluminum must not exceed a certain limited quantity.

The invention, therefore, has for its object to minimize

2

the detrimental effect of metallic aluminum, by keeping the ratio between aluminum and aluminum nitride at a specified value, and by keeping the free nitrogen content under 0.004% by weight.

Thus, the present invention relates to low-Mn grade steels containing about 0.05 to 0.25% carbon, less than about 0.60% silicon, about 1.00 to 2.50% manganese, which are characterized by a component consisting of about 0.03 to 0.12% precipitated aluminum nitride, and 10 a component consisting of about 0.003 to 0.15% dissolved metallic aluminum, as well as featuring the granular structure wherein the grain size is over No. 9 in terms of the ASTM ferrite grain size number system. The invention further comprises steels of the composition containing 0.05—0.25% carbon, less than 0.60% silicon, 1.00—2.5% manganese, 0.03—0.12% precipitated aluminum nitride, 0.003—0.15% metallic aluminum in solid solution, and 1% of at least one of the elements of the group consisting of nickel, chromium, molybdenum, 20 vanadium and copper, and less than 0.1% boron.

The foregoing percentages are by weight, and the balance of the steel is iron with incidental impurities.

In the following, the full details of the present invention will be disclosed, in which references will be made 25 to figures and photographs, where,

FIGS. 1 and 2 are drawings in which the transition temperature characteristics of various low-Mn grade steels are compared in terms of Charpy V-notch testing method,

30 FIG. 3 is a drawing to show the relation between the amount of dissolved metallic aluminum in solid solution and the ferrite grain size,

FIG. 4 is a drawing to show the relation between the amount of precipitated aluminum nitride and the ferrite 35 grain size for various low-Mn grade steels with different amounts of dissolved metallic aluminum in solid solution,

FIGS. 5 and 6 are photomicrograms to show the granular structure of a low-Mn grade steel of the present invention.

The chemical composition of low-Mn grade steels representative for those that were submitted to various tests is summarized in Table 1. The mechanical properties of said steels are listed in Table 2.

Table I

| Specimen No.     | C    | Si   | Mn   | P     | S     | Ni   | Cr   | Mo   | V    |
|------------------|------|------|------|-------|-------|------|------|------|------|
| LMn 1            | 0.09 | 0.31 | 1.35 | 0.020 | 0.030 | —    | —    | —    | —    |
| LMn 2            | 0.13 | 0.49 | 1.35 | 0.013 | 0.007 | —    | —    | —    | —    |
| LMn 3            | 0.09 | 0.37 | 1.17 | 0.017 | 0.007 | —    | —    | —    | —    |
| LMn 4            | 0.12 | 0.31 | 1.45 | 0.014 | 0.009 | 0.47 | 0.33 | 0.12 | 0.07 |
| Commercial LMn A | 0.13 | 0.22 | 1.20 | 0.014 | 0.010 | —    | —    | —    | —    |
| Commercial LMn B | 0.14 | 0.42 | 1.12 | 0.017 | 0.023 | —    | —    | —    | —    |
| Commercial LMn C | 0.12 | 0.35 | 1.13 | 0.016 | 0.006 | 0.55 | 0.26 | —    | 0.12 |

| Specimen No.     | Total Al | Total N | AlN   | Al <sub>2</sub> O <sub>3</sub> | Metallic Al | Free N | Remarks                                 |
|------------------|----------|---------|-------|--------------------------------|-------------|--------|-----------------------------------------|
| LMn 1            | 0.086    | 0.024   | 0.067 | 0.015                          | 0.034       | 0.002  | Si-Mn type high-tension steel.          |
| LMn 2            | 0.113    | 0.030   | 0.078 | 0.016                          | 0.053       | 0.004  | Do.                                     |
| LMn 3            | 0.203    | 0.023   | 0.061 | 0.023                          | 0.151       | 0.003  | Do.                                     |
| LMn 4            | 0.176    | 0.033   | 0.085 | 0.027                          | 0.106       | 0.003  | Si-Mn-Ni-Cr-Mo type high-tension steel. |
| Commercial LMn A | 0.055    | 0.009   | 0.024 | 0.013                          | 0.032       | 0.001  | Si-Mn type high-tension steel.          |
| Commercial LMn B | 0.045    | 0.011   | 0.024 | 0.005                          | 0.026       | 0.003  | Do.                                     |
| Commercial LMn C | 0.032    | 0.009   | 0.021 | 0.011                          | 0.012       | 0.002  | Si-Mn-Ni-Cr-V type high-tension steel.  |

Table 2

| Specimen No. | Heat treatment | Test piece diameter, mm. | Guage length, mm. | Yield point, kg./mm. <sup>2</sup> | Tensile strength, kg./mm. <sup>2</sup> | Yield ratio, percent | Elongation, percent | Reduction of area, percent | Fracture position |
|--------------|----------------|--------------------------|-------------------|-----------------------------------|----------------------------------------|----------------------|---------------------|----------------------------|-------------------|
| LMn 1        | N*             | 10                       | 40                | 45.2                              | 52.6                                   | 85.9                 | 33.8                | 71.9                       | A                 |
| LMn 2        | Q, T†          | 10                       | 40                | 48.3                              | 58.3                                   | 82.8                 | 32.5                | 78.5                       | A                 |
| LMn 3        | N              | 10                       | 40                | 43.2                              | 57.6                                   | 75.0                 | 31.0                | 67.5                       | A                 |
| LMn 4        | Q, T           | 10                       | 40                | 51.5                              | 63.2                                   | 81.5                 | 23.5                | 73.0                       | B                 |
| LMn A        | N              | 10                       | 40                | 44.3                              | 53.5                                   | 82.8                 | 35.9                | 70.4                       | A                 |
| LMn B        | Q, T           | 14                       | 50                | 47.8                              | 57.9                                   | 82.6                 | 34.3                | 70.9                       | A                 |
| LMn C        | N              | 14                       | 50                | 54.3                              | 64.9                                   | 83.7                 | 22.5                | 73.1                       | A                 |
|              |                |                          |                   | 52.4                              | 58.4                                   | 89.7                 | 24.0                |                            | A                 |
|              |                |                          |                   | 36.7                              | 53.5                                   | 68.7                 | 29.0                |                            | A                 |
|              |                |                          |                   | 52.9                              | 63.9                                   | 82.8                 | 22.0                |                            | A                 |

\*Normalized. †Quench-and-Tempered.

A brief comment on the nature of steels presented in the above tables is now in order. Steels designated as LMn 1 to 4 are the ones in accordance with the present invention. The LMn 1 is a Si-Mn type high-tension steel containing an amount of precipitated aluminum nitride and dissolved metallic aluminum in solid solution that exhibits tensile strengths of the order of 50 and 55 kg./mm.<sup>2</sup> when normalized or quench-and-tempered, respectively. The LMn 2 has a similar composition to LMn 1 except for the carbon content which is slightly higher than in LMn 1, and as a consequence, its tensile strengths are of the order of 55 and 60 kg./mm.<sup>2</sup> corresponding to mode of heat treatment of normalization or quench-and-tempering, respectively. LMn 3 is a similar steel to LMn 1 except that its metallic aluminum component is considerably higher than in LMn 1, and the tensile strengths are almost equal to those of the latter. LMn 4 is again another Si-Mn type steel except modified by small amounts of Ni, Cr, Mo and V each to improve the tensile strengths which are of the order of 60 or 70 kg./mm.<sup>2</sup> when normalized or quench-and-tempered, respectively.

Steels designated as LMn A, LMn B and LMn C are so-called low-Mn grade steels that were acquired from commercial market. The LMn A is equivalent to LMn 2, LMn B to LMn 1, and LMn C to LMn 4, respectively.

The transition temperature curves obtained from low-Mn grade steels of the present invention and those from commercial steels of the same grade are compared in FIG. 1. It will be seen from said figure that the low-Mn grade steels containing precipitated aluminum nitride of more than 0.03% all have transition temperature curves that are in a temperature region that is lower by about 40° to 80° C. as compared with those of commercial counterparts, and, moreover, the absorbed energy at fracture in the former varieties is far larger than that in the latter at any temperature tested.

It will be noted in FIG. 1, furthermore, that the transition temperature curves of LMn 3 is shifted towards the higher temperature side with respect to those of LMn 1. The relative shift of the curve is about 35° C. and about 45° C. for the cases of normalization and quench-and-tempering, respectively. Thus, the brittleness of LMn 3 is evident with regard to LMn 1 in either state of heat treatment. Since no major difference in chemical composition is to be detected except for the amount of dissolved metallic aluminum between these two steels as may be judged from Table 1, a conclusion that such embrittlement as mentioned above should be attributed to the excessive amount of dissolved metallic aluminum in LMn 3 is proper.

FIG. 3 shows a relationship between ferrite grain size and amount of dissolved metallic aluminum in solid solution, while FIG. 4 shows a relation between ferrite grain size and amount of precipitated aluminum nitride for different amounts of dissolved metallic aluminum in solid solution, the ferrite grain size being reckoned in terms of the ASTM ferrite grain size number system in either case. It will be noted that for the grain size of these steels to be over No. 9, an amount of 0.1% or 0.23% for dis-

solved metallic aluminum represents the upper limit in cases of normalization and quench-and-tempering, respectively. The amount of precipitated aluminum nitride, on the other hand, must be more than 0.035% or 0.0075% in cases of normalization and quench-and-tempering, respectively, to obtain a refined granular structure of over No. 9 in terms of the above-mentioned grain size system, provided that the quantity of dissolved metallic aluminum is small. It will be further seen that, for steels containing a large amount of dissolved metallic aluminum, the necessary limitation imposed upon the content of precipitated aluminum nitride is over 0.10% or 0.05% corresponding to the mode of heat treatment of normalization or quench-and-tempering, respectively.

It follows from those empirical findings described above, and the fact that the cooling rates applied on specimens involved in the various tests were rather faster than what would be realized in practice, a use of optimum compositions ranging from about 0.03 to 0.12% for precipitated aluminum nitride, and from about 0.003 to 0.15% for dissolved metallic aluminum in solid solution, is proper for successful production of fine-grained, low-temperature ductile low-Mn grade steels.

In FIG. 2, the transition temperature characteristics of two different low-Mn grade steels, as normalized, one due to the present invention, the LMn 4, and the other a commercial steel, the LMn C, are compared. It is to be seen that the steel of the present invention is far more ductile than its commercial counterpart as evidenced by the relative position of the transition temperature curves, the one representing the steel to in accordance with the present invention lying at far lower side in the temperature scale and far above along the impact value scale with respect to the commercial steel.

FIGS. 5 and 6 are photomicrograms showing the microstructure of a low-Mn grade steel of the present invention, the LMn 1. It is to be noted the grain size thereof is about No. 12 in terms of the ASTM ferrite grain size system.

The low-Mn grade steels due to the present invention are all heat-treatable in that the granular structure thereof can be refined further, hence the low-temperature ductility more improved, as compared with the same stock but in a state of as-rolled or as-forged, by executing a heat treatment process consisting of rapidly cooling said steel from a temperature within a temperature range of maximum precipitation of aluminum nitride, to be followed, if desired, by reheating it to a lower temperature for tempering.

The temperature of maximum precipitation of aluminum nitride is about 800° C. to 1050° C., whereafter the steel is rapidly cooled in a fluid medium to retain the state of precipitation to the fullest extent. If desired, the steel may be further subjected to a tempering step at a temperature between about 150° C. and 750° C.

I claim:

1. A nitride bearing low manganese ductile steel consisting essentially of, by weight, 0.05% to 0.15% carbon, less than 0.60% silicon, 1.0% to 2.5% manganese, 0.03%

to 0.12% aluminum nitride, 0.003% to 0.15% metallic aluminum in solid solution, balance iron with incidental impurities, said steel having a grain size finer than number 9 in terms of the ASTM ferrite grain size numbering system.

2. A nitride bearing low manganese ductile steel consisting essentially of, by weight, 0.05% to 0.15% carbon, less than 0.60% silicon, 1.0% to 2.5% manganese, 0.03% to 0.12% precipitated aluminum nitride, 0.003% to 0.15% metallic aluminum in solid solution, less than 1% of at least one element selected from the group consisting of nickel, chromium, molybdenum, vanadium, and copper, less than 0.1% boron, balance iron with incidental impurities said steel having a grain size finer than number 9 in terms of the ASTM ferrite grain size numbering system.

3. Method for the heat treatment of steel having a chemical composition according to claim 1, comprising the steps of heating said steel to a temperature between about 800° and 1050° C. for maximum precipitation of aluminum nitride, and then cooling the steel rapidly in a fluid medium to retain the state of precipitation of the nitride to the fullest extent.

4. Method for the heat treatment of steel having a chemical composition according to claim 2, comprising the steps of heating said steel to a temperature between about 800° and 1050° C. for maximum precipitation of aluminum nitride, and then cooling the steel rapidly in

a fluid medium to retain the state of precipitation of the nitride to the fullest extent.

5. The method of claim 3 in which the steel is further subjected to a tempering step at a temperature between about 150° and 750° C.

6. The method of claim 4 in which the steel is further subjected to a tempering step at a temperature between about 150° and 750° C.

10

References Cited by the Examiner

UNITED STATES PATENTS

2,679,454 5/54 Offenhauer ----- 75-128.5

15

FOREIGN PATENTS

808,556 2/59 Great Britain.

20

OTHER REFERENCES

Geil et al.: Journal of Research of the National Bureau of Standards, vol. 48, No. 3, March 1952, pages 193-200.

Case et al.: Al In Iron and Steel, 1953, pages 79-89 and 130-132; published by John Wiley and Sons, Inc., New York, N.Y.

25

DAVID L. RECK, Primary Examiner.

MARCUS U. LYONS, ROGER L. CAMPBELL,  
HYLAND BIZOT, Examiners.